# EUROPEAN PATENT APPLICATION

(11) **EP 4 787 407 A1**
(43) Date of publication of application: **05.08.2026**
(21) Application number: 24870078.3
(22) Date of filing: 31.07.2024
(51) Int. Cl.: H01F 1/057

(54) **HIGH-TEMPERATURE-RESISTANT SINTERED NEODYMIUM-IRON-BORON MAGNET, PREPARATION METHOD THEREFOR, AND USE THEREOF**

(30) Priority: 28.09.2023 CN 202311275411
(71) Applicant: Yantai Zhenghai Magnetic Material Co., Ltd., Yantai Shandong 264006 (CN)
(72) Inventor: PENG, Buzhuang, Yantai, Shandong 264006 (CN); ZHANG, Yumeng, Yantai, Shandong 264006 (CN); YANG, Kai, Yantai, Shandong 264006 (CN); QIAN, Yi, Yantai, Shandong 264006 (CN); ZHANG, Ting, Yantai, Shandong 264006 (CN)
(74) Representative: Gille Hrabal Partnerschaftsgesellschaft mbB Patentanwälte
(86) International application number: PCT/CN2024/108769
(87) International publication number: WO 2025/066525

(57) **Abstract**

Disclosed in the present invention are a high-temperature-resistant sintered neodymium-iron-boron magnet, a preparation method therefor, and the use thereof. The magnet is represented by R-Fe-B-M, and comprises on the basis of mass percentages, 100% in total: 29wt%-35wt% of R, R being a rare earth element, 0.9wt%-1.3wt% of B, and less than 5 wt% of M, M being selected from one or more of Ti, V, Cr, Mn, Co, Ga, Cu, Si, Al, Zr, Nb, W and Mo, with the balance being iron and unavoidable impurities. Crystal grains of the sintered neodymium-iron-boron magnet of the present invention have a smaller dimensional change rate in different directions at high temperatures, such that the probability of forming demagnetizing fields is reduced and the coercivity of the neodymium-iron-boron magnet at high temperatures is improved, thereby improving the characteristic of resisting demagnetization at high temperatures of the sintered neodymium-iron-boron magnet.

## Description

**The present application claims priority to the Patent Application No.** 202311275411.7, entitled "HIGH-TEMPERATURE-RESISTANT SINTERED NEODYMIUM-IRON-BORON MAGNET, PREPARATION METHOD THEREFOR, AND USE THEREOF", filed with the China National Intellectual Property Administration on September 28, 2023**, which is incorporated herein by reference in its entirety.**

### TECHNICAL FIELD

The present disclosure relates to the technical field of NdFeB-based sintered magnets, and in particular, relates to a high-temperature-resistant sintered neodymium-iron-boron magnet, a preparation method therefor, and use thereof.

### BACKGROUND

Since the advent of sintered permanent magnet materials (or sintered neodymium-iron-boron magnets), they have rapidly been widely used in numerous fields such as electronics, energy, communications, instruments, and the like due to their excellent magnetic properties and relatively high cost-effectiveness. In recent years, permanent magnet materials have been increasingly widely used in the field of automobiles. However, an automobile motor will generate a high temperature when working, and the permanent magnet material will be demagnetized at the high temperature, resulting in a decrease in the performance of the permanent magnet material.

In order to solve the problem of high-temperature demagnetization of the permanent magnet material, in addition to the optimization and upgrade of the motor cooling system, improving the coercivity of the permanent magnet material is a more effective way to solve the high-temperature demagnetization of the permanent magnet material.

At present, there are three main methods for improving the coercivity of a permanent magnet. The first method is to increase an anisotropic field of the magnet by adding a heavy rare earth element, such as dysprosium (Dy), terbium (Tb), or holmium (Ho), thereby improving the coercivity of the magnet. The second method is a grain refinement technique. As the grain dimension decreases, the internal defects of the grains decrease, the internal demagnetization field decreases, and the coercivity of the magnet increases. The third method is a grain boundary diffusion technique. This technique enables heavy rare earths to diffuse along the grain boundary, significantly increases the anisotropy constant at the grain boundary, and achieves a significant increase in the coercivity of the magnet under the condition that a small amount of heavy rare earth is used.

In order to meet the high-temperature demagnetization requirements of existing automobile motors, more or less heavy rare earth elements are used in the three methods described above. With the rising price of heavy rare earth in recent years, the production of permanent magnet materials with higher temperature resistance and reduced usage of heavy rare earth is a key research direction for various enterprises.

### SUMMARY

After conducting intensive studies on the problems described above, the inventors found that the sintered neodymium-iron-boron magnet has the characteristic of anisotropy, which is manifested not only in the orientation of the magnetic field but also in the expansion coefficient. The sintered neodymium-iron-boron magnet has different coefficients of thermal expansion in different directions. For example, in the direction of an easy magnetization axis (the orientation direction of the magnet), it externally exhibits expansion as the temperature increases; in the direction of a hard magnetization axis (perpendicular to the orientation direction of the magnet), it externally exhibits contraction as the temperature increases. Due to the difference in expansion proportions in different directions, grains of the sintered neodymium-iron-boron magnet change at a high temperature, and this change may cause a demagnetization field, resulting in a decrease in the coercivity of the neodymium-iron-boron magnet at a high temperature.

In order to overcome the defects in the prior art, the present disclosure provides a high-temperature-resistant sintered neodymium-iron-boron magnet, wherein the magnet is represented by R-Fe-B-M and comprises, based on a mass ratio of 100%,
29 wt% to 35 wt% of R, wherein R is a rare earth element;
0.9 wt% to 1.3 wt% of B;
less than 5 wt% of M, wherein M is selected from one or more of Ti, V, Cr, Mn, Co, Ga, Cu, Si, Al, Zr, Nb, W, and Mo;
the balance is iron and inevitable impurities.

According to an embodiment of the present disclosure, R is selected from at least one of lanthanum (La), cerium (Ce), praseodymium (Pr), neodymium (Nd), promethium (Pm), samarium (Sm), europium (Eu), gadolinium (Gd), terbium (Tb), dysprosium (Dy), holmium (Ho), erbium (Er), thulium (Tm), ytterbium (Yb), lutetium (Lu), scandium (Sc), and yttrium (Y). Preferably, R is praseodymium (Pr) and neodymium (Nd).

According to an embodiment of the present disclosure, the magnet comprises, based on a mass ratio of 100%, 30 wt% to 33 wt% of R, wherein R is a rare earth element;
0.9 wt% to 1.1 wt% of B;
0.5 wt% to 4.5 wt% of M, wherein M is selected from one or more of Ti, V, Cr, Mn, Co, Ga, Cu, Si, Al, Zr, Nb, W, and Mo;
the balance is iron and inevitable impurities.

In the present disclosure, a reference temperature is set as T₀ (for example, the temperature is normal temperature; for another example, the temperature is 20 °C), and a measurement temperature is set as T (°C). A magnet dimension L₀ is measured at T₀, and a magnet dimension L(T) is measured after heating the magnet to the temperature T; T - T₀ = ΔT, L(T) - L₀ = ΔL. A linear expansion coefficient C of the sintered neodymium-iron-boron magnet is calculated by C = [△L/L₀]/△T. The linear expansion coefficient comprises: a linear expansion coefficient C1 parallel to a magnetizing direction of the magnet; a linear expansion coefficient C2 perpendicular to the magnetizing direction and parallel to a pressing direction; a linear expansion coefficient C3 in the other direction perpendicular to the magnetizing direction; a mean value C4 of the linear expansion coefficients in two directions perpendicular to the magnetizing direction.

According to an embodiment of the present disclosure, the linear expansion coefficient C1 parallel to the magnetizing direction of the magnet is (5 to 8) × 10⁻⁶/°C,
the linear expansion coefficient C2 perpendicular to the magnetizing direction and parallel to the pressing direction is (-3 to -0.6) × 10⁻⁶/°C,
the linear expansion coefficient C3 in the other direction perpendicular to the magnetizing direction is (-4 to -1) × 10⁻⁶/°C,
and the mean value C4 of the linear expansion coefficients in two directions perpendicular to the magnetizing direction is (-3.5 to -0.8) × 10⁻⁶/°C, wherein C4 = (C2 + C3)/2;
and, 1.5 ≤ |C1/C4| ≤ 8.

In the present disclosure, as the temperature increases, the sintered neodymium-iron-boron magnet shows expansion in a direction parallel to the magnetizing direction of the magnet and contraction in the other two directions perpendicular to the magnetizing direction. Therefore, C1 is greater than 0, C2 is less than 0, and C3 is less than 0.

The present disclosure also provides a preparation method for the sintered neodymium-iron-boron magnet described above, which comprises:
(1) preparing an R-Fe-B-M alloy flake from respective starting materials by a rapid hardening and strip casting method;
(2) subjecting the alloy flake to hydrogenation treatment by introducing hydrogen; after completion of the hydrogenation treatment, performing heating to a temperature of 250 to 350 °C for dehydrogenation treatment; after completion of the dehydrogenation, introducing argon to not less than 30 kPa, and performing heating and heat preservation; after completion of the heat preservation, performing cooling to obtain an alloy powder;
(3) subjecting the alloy powder in step (2) to jet milling to obtain a magnetic powder, and performing pressing, sintering, and tempering treatments to obtain the magnet.

According to an embodiment of the present disclosure, in step (1), the rapid hardening and strip casting method is a technique well known in the art.

According to an embodiment of the present disclosure, in step (2), a hydrogen absorption pressure for the hydrogenation treatment is 100 to 200 kPa, preferably 140 to 180 kPa, and a hydrogen absorption time is 30 to 180 min, preferably 90 to 150 min.

According to an embodiment of the present disclosure, in step (2), a dehydrogenation time is 180 to 360 min.

According to an embodiment of the present disclosure, in step (2), a dehydrogenation temperature is 250 °C, 260 °C, 270 °C, 280 °C, 290 °C, 300 °C, 310 °C, 320 °C, 330 °C, 340 °C, or 350 °C. According to an embodiment of the present disclosure, in step (2), argon is introduced to not less than 30 kPa, e.g., 30-60 kPa, after completion of the dehydrogenation. Illustratively, argon is introduced to 30 kPa, 35 kPa, 40 kPa, 45 kPa, 50 kPa, 5 kPa, or 60 kPa.

According to an embodiment of the present disclosure, in step (2), a heat preservation temperature is 700-800 °C, e.g., 720 °C, 740 °C, 760 °C, 780 °C, or 800 °C.

According to an embodiment of the present disclosure, in step (2), a heat preservation time is 60 to 180 min.

According to an embodiment of the present disclosure, in step (2), during the cooling, an argon pressure is ≥ 20 kPa, e.g., 20-60 kPa, at a temperature of not less than 350 °C. Illustratively, the argon pressure is 20 kPa, 30 kPa, 40 kPa, 50 kPa, or 60 kPa.

According to an embodiment of the present disclosure, in step (3), the alloy powder in step (2) is mixed with a lubricant and subjected to jet milling to obtain the magnetic powder.

According to an embodiment of the present disclosure, in step (3), a granularity D50 of the magnetic powder is 2 to 5 µm.

According to an embodiment of the present disclosure, in step (3), a content of the lubricant is 0.03 to 0.5 wt% , preferably 0.05 to 0.1 wt%, of the alloy powder in step (2).

According to an embodiment of the present disclosure, in step (3), the magnetic powder is press-molded under a magnetic field orientation. Preferably, the orientation magnetic field is 1.5 to 2.5 T. According to an embodiment of the present disclosure, in step (3), a sintering temperature is 800 to 1200 °C, preferably 900 to 1080 °C, and a heat preservation time is 3 to 20 h, preferably 3 to 8 h.

According to an embodiment of the present disclosure, in step (3), the tempering treatment is two-stage tempering, for example, two-stage tempering in a vacuum tempering furnace; a primary tempering temperature is 700 to 900 °C, and a heat preservation time is 3 to 7 h; a secondary tempering temperature is 450 to 600 °C, and a heat preservation time is 3 to 7 h.

According to an embodiment of the present disclosure, the method further comprises step (4): performing grain boundary diffusion treatment on the magnet, wherein a diffusion source is at least one of heavy rare earth Dy, Tb, Ho, Nd, and Pr.

According to an embodiment of the present disclosure, in step (4), a content of the diffused heavy rare earth is 0.1-1.5 wt%, preferably 0.2-1.2 wt%.

According to an embodiment of the present disclosure, in step (4), a diffusion temperature is 800 to 950 °C, and a diffusion time is at least 3 h, preferably 3-30 h.

According to an embodiment of the present disclosure, in step (4), a grain boundary diffusion treatment method may be at least one of a thermal spraying method, a coating method, a sputtering method, an impregnation method, and the like.

According to an embodiment of the present disclosure, in step (4), the magnet may be further subjected to treatments such as degreasing, acid washing, and the like before the diffusion treatment. As an exemplary implementation method of the present disclosure, the preparation method for the high-temperature-resistant sintered neodymium-iron-boron magnet specifically comprises:
1) obtaining an R-Fe-B-M alloy flake by a rapid hardening and strip casting method;
2) subjecting the alloy flake described above to hydrogenation treatment, with a hydrogen absorption pressure being 100 to 200 kPa and a hydrogen absorption time being 30 to 180 min; after completion of the hydrogen absorption, performing heating to a temperature of 250 to 350 °C for dehydrogenation treatment for a dehydrogenation time of 180 to 360 min; after completion of the dehydrogenation, introducing argon to not less than 30 kPa, and performing heating to a temperature of 700 to 800 °C, with a heat preservation time being 60 to 180 min; after completion of the heat preservation, performing cooling, wherein during the cooling, an argon pressure is ≥ 20 kPa at a temperature of not less than 350 °C;
3) mixing the alloy powder described above with a lubricant and performing jet milling treatment to obtain a magnetic powder; press molding the magnetic powder under the magnetic field orientation, wherein the orientation magnetic field is 1.5 to 2.5 T;
4) subjecting the compact described above to sintering treatment in a vacuum sintering furnace at a sintering temperature of 900 to 1080 °C for a sintering time of 3 to 8 h; after completion of heat preservation, performing cooling to ≤ 200 °C, and performing primary tempering treatment at 700 to 900 °C, with a heat preservation time being 3-7 h; performing secondary tempering treatment at 450-600 °C, with a heat preservation time being 3-7 h, to obtain the sintered neodymium-iron-boron magnet;
5) performing diffusion treatment on the magnet in step 4): processing the magnet in step 4) to a desired dimension, and performing grain boundary diffusion treatment after degreasing and acid washing treatments, wherein a diffusion temperature is 800 to 950 °C, a diffusion time is at least 3 h, and a diffusion source is at least one element of Dy, Tb, Ho, Nd, and Pr.

The present disclosure also provides use of the sintered neodymium-iron-boron magnet described above in the fields of new energy automobile industry and wind power generation.

### Beneficial Effects of Present Disclosure:

The grains of the sintered neodymium-iron-boron magnet of the present disclosure have a smaller dimensional change rate in different directions at a high temperature, which reduces the probability of forming a demagnetization field and improves the coercivity of the neodymium-iron-boron magnet at a high temperature, thereby improving the demagnetization resistance of the sintered neodymium-iron-boron magnet at a high temperature.

### BRIEF DESCRIPTION OF THE DRAWINGS

FIG. 1 is a graph showing the linear expansion coefficient C1 parallel to the magnetizing direction of the magnet tested in Example 1;
FIG. 2 is a graph showing the linear expansion coefficient C2 perpendicular to the magnetizing direction and parallel to the pressing direction tested in Example 1;
FIG. 3 is a graph showing the linear expansion coefficient C3 in the other direction perpendicular to the magnetizing direction tested in Example 1.

### DETAILED DESCRIPTION

The technical solutions of the present disclosure are further described in detail below with reference to specific examples. It will be appreciated that the following examples are merely exemplary illustrations and explanations of the present disclosure and should not be construed as limiting the claimed scope of the present disclosure. All techniques implemented on the basis of the content described above of the present disclosure fall within the claimed scope of the present disclosure.

Unless otherwise stated, the starting materials and reagents used in the following examples are all commercially available products or can be prepared by using known methods.

Measurement of the linear expansion coefficient of sintered neodymium-iron-boron magnet of the present disclosure:
The linear expansion coefficient was determined using a thermomechanical analyzer (model: TMA402F3). The method used is static thermomechanical analysis, which measures the deformation of a material as a function of temperature under a non-oscillating load, with programmed temperature control. The test temperature was from 20 °C to a high temperature at a ramping rate of 3-5 °C/min.

The test directions are the three directions of the magnet.

### Example 1. Comparative Examples 1-7

Preparation is performed according to the following method. The alloy flake was prepared by subjecting at least 99% purity by weight of NdPr, Co, Al, Fe, Cu, Ga, Ti, and ferroboron to highfrequency melting in an argon atmosphere and casting the resulting melt onto a quenching roller. The contents of the respective starting materials are 31.5% NdPr, 1.0% Co, 0.5% Al, 0.2% Cu, 0.2% Ga, 0.18% Ti, and 0.98% B, respectively, with the balance being Fe and inevitable impurities.

The alloy flake was subjected to hydrogenation treatment, with a hydrogen absorption pressure being 180 kPa and a hydrogen absorption time being 120 min. After completion of the hydrogen absorption, the alloy flakes were treated according to the hydrogenation treatment process of alloy flakes in Table 1 and crushed into coarse powders. Then, the coarse powder was subjected to jet mill grinding to obtain a magnetic powder with a granularity D50 of 4.0 µm. The jet-milled powder described above was mixed with 0.3 wt% of a lubricant for 2 h, and press-molding was performed at normal temperature in an orientation field with a magnetic field intensity of 2 T. Then, the blank was put into a vacuum sintering furnace and sintered at 1030 °C for 6 h. After completion of heat preservation, the blank was cooled to 100 °C. Then, the blank was heated to 900 °C and subjected to primary tempering treatment at 900 °C for 3 h. Secondary tempering treatment was then performed at 520 °C for 5 h. The blank was cooled and taken out of the furnace, thus obtaining a neodymium-iron-boron magnet.

The neodymium-iron-boron magnet obtained above was processed into a product with a dimension of 10-8-6 mm, and the linear expansion coefficients of the product in different directions were tested using a thermomechanical analyzer. The ramping rate was 5 °C/min, and the test temperature was 20-140 °C. The test results are shown in Table 2.

In addition, the neodymium-iron-boron magnet obtained above was processed into a D10-10 mm product, and magnetic tests were performed at 20 °C and 140 °C. The test results are shown in Table 3.

**Table 1. Hydrogenation processes corresponding to Example 1 and Comparative Examples 1-7**

| | Alloy flake hydrogenation treatment process | | | | |
|---|---|---|---|---|---|
| | Dehydrogenation temperature (°C) | Argon pressure introduced after completion of dehydrogenation (kPa) | Heat preservation temperature (°C) | Heat preservation time (min) | Argon pressure introduced during cooling at temperature of not less than 350 °C (kPa) |
| Example 1 | 300 | 45 | 750 | 120 | 30 |
| Comparative Example 1 | 450 | 45 | 750 | 120 | 30 |
| Comparative Example 2 | 200 | 45 | 750 | 120 | 30 |
| Comparative Example 3 | 300 | 0 | 750 | 120 | 30 |
| Comparative Example 4 | 300 | 10 | 750 | 120 | 30 |
| Comparative Example 5 | 300 | 45 | 600 | 150 | 30 |
| Comparative Example 6 | 300 | 45 | 900 | 100 | 30 |
| Comparative Example 7 | 300 | 45 | 750 | 120 | 15 |

The products prepared in Example 1 and Comparative Examples 1-7 were subjected to a linear expansion coefficient test. The linear expansion coefficient test method was as follows:
The magnet dimension was measured as L₀ at normal temperature T₀. The magnet temperature was raised to a measurement temperature T (°C), and the magnet dimension L(T) is measured; T - T₀ = △T, L(T) - L₀ = △L. The linear expansion coefficient C of the sintered neodymium-iron-boron magnet was calculated by C = [△L/L₀]/△T.

The test results are shown in Table 2 below.

**Table 2. Tested linear expansion coefficients of neodymium-iron-boron products corresponding to Example 1 and Comparative Examples 1-7**

| | C1 (10⁻⁶/°C) | C2 (10⁻⁶/°C) | C3 (10⁻⁶/°C) | C4 (10⁻⁶/°C) | \|C1/C4\| |
|---|---|---|---|---|---|
| Example 1 | 5.56 | -2.69 | -2.93 | -2.71 | 2.05 |
| Comparative Example 1 | 7.87 | -0.63 | -1.11 | -0.87 | 9.05 |
| Comparative Example 2 | 8.93 | -0.44 | -0.88 | -0.66 | 13.53 |
| Comparative Example 3 | 9.85 | -0.49 | -0.82 | -0.655 | 15.04 |
| Comparative Example 4 | 8.47 | -0.52 | -0.95 | -0.735 | 11.52 |
| Comparative Example 5 | 7.42 | -0.74 | -1.02 | -0.88 | 8.43 |
| Comparative Example 6 | 7.67 | -0.71 | -1.07 | -0.89 | 8.55 |
| Comparative Example 7 | 7.80 | -0.66 | -1.09 | -0.875 | 8.91 |

The products prepared in Example 1 and Comparative Examples 1-7 were subjected to Br, Hcj (including 20 °C and 140 °C), and Hcj temperature coefficient tests. The test results are shown in Table 3 below.

**Table 3. Magnetic property results of neodymium-iron-boron products in Example 1 and Comparative Examples 1-7**

| | Br(T) 20°C | Hcj(kA/m) 20°C | Hcj(kA/m) 140°C | Hcj temperature coefficient |
|---|---|---|---|---|
| Example 1 | 1.36 | 1569 | 559 | -0.536 |
| Comparative Example 1 | 1.361 | 1495 | 526 | -0.540 |
| Comparative Example 2 | 1.345 | 1556 | 517 | -0.556 |
| Comparative Example 3 | 1.365 | 1423 | 475 | -0.555 |
| Comparative Example 4 | 1.363 | 1460 | 497 | -0.550 |
| Comparative Example 5 | 1.36 | 1531 | 537 | -0.541 |
| Comparative Example 6 | 1.365 | 1437 | 500 | -0.543 |
| Comparative Example 7 | 1.359 | 1488 | 525 | -0.539 |

As can be seen from the comparison of the data of Example 1 and Comparative Example 1, the dehydrogenation temperature in Comparative Example 1 was excessively high and exceeded the range required by the patent process. Although C1, C2, C3, and C4 were all within the ranges, these values were all within the critical ranges, resulting in |C1/C4| exceeding the patent ranges, leading to deteriorated temperature resistance (deteriorated Hcj temperature coefficient). Meanwhile, due to the excessively high dehydrogenation temperature, the normal temperature Hcj of Comparative Example 1 was relatively low. In addition, due to the deteriorated temperature resistance, the high temperature Hcj became even lower.

As can be seen from the comparison of the data of Example 1 and Comparative Example 2, the dehydrogenation temperature in Comparative Example 2 was excessively low, resulting in C1, C2, C3, C4, and |C1/C4| all exceeding the patent ranges, leading to deteriorated temperature resistance (deteriorated Hcj temperature coefficient). In addition, due to the excessively low dehydrogenation temperature, the normal temperature Br of Comparative Example 2 was significantly reduced. This process also increased the hydrogen content before sintering, leading to more cracks in the product after sintering and an increase in the product defect rate.

As can be seen from the comparison of the data of Example 1, Comparative Example 3, and Comparative Example 4, the argon pressure introduced after completion of dehydrogenation in Comparative Example 3 was 0, i.e., no argon was introduced. The argon pressure introduced after completion of dehydrogenation in Comparative Example 4 was 10 kPa, which was relatively low. In both comparative examples, dehydrogenation of the alloy flake occurred at a subsequent temperature of 750 °C, resulting in a poor crushing effect of the alloy flake, which consequently resulted in C1, C2, C3, C4, and |C1/C4| all exceeding the patent ranges, leading to deteriorated temperature resistance (deteriorated Hcj temperature coefficient). In addition, due to the excessively deteriorated linear expansion coefficient, excessive defects were generated in the product during sintering and cooling, resulting in relatively low normal temperature Hcj in Comparative Example 3 and Comparative Example 4. In addition, due to the deteriorated temperature resistance, the high temperature Hcj became even lower.

As can be seen from the comparison of the data of Example 1 and Comparative Example 5, due to the excessively low heat preservation temperature in Comparative Example 5, the transition of elements between the grains and the grain boundaries was insufficient, and the structure presented a metastable state. Although C1, C2, C3, and C4 were all within the ranges, these values were all within the critical ranges, resulting in |C1/C4| exceeding the patent ranges, leading to deteriorated temperature resistance (deteriorated Hcj temperature coefficient).

As can be seen from the comparison of the data of Example 1 and Comparative Example 6, the heat preservation temperature in Comparative Example 6 was excessively high, leading to grain growth in the alloy flake to a certain extent, resulting in a deteriorated crushing effect of the alloy flake. Although C1, C2, C3, and C4 were all within the ranges, these values were all within the critical ranges, resulting in |C1/C4| exceeding the patent ranges, leading to deteriorated temperature resistance (deteriorated Hcj temperature coefficient). In addition, due to grain growth in the alloy flake, the normal temperature Hcj of the product was reduced. In addition, due to the deteriorated temperature resistance, the high temperature Hcj became even lower.

As can be seen from the comparison of the data of Example 1 and Comparative Example 7, the argon pressure introduced during the cooling at a temperature of not less than 350 °C in Comparative Example 7 was excessively low, leading to dehydrogenation of the alloy flake at a relatively high temperature. Although C1, C2, C3, and C4 were all within the ranges, these values were all within the critical ranges, resulting in |C1/C4| exceeding the patent ranges, leading to deteriorated temperature resistance (deteriorated Hcj temperature coefficient). In addition, due to dehydrogenation at a relatively high temperature in Comparative Example 7, the normal temperature Hcj of the product in Comparative Example 7 was relatively low. In addition, due to the deteriorated temperature resistance, the high temperature Hcj became even lower.

### Example 2

The neodymium-iron-boron magnet prepared in Example 1 was processed into a square piece with a dimension of 20-15-3 mm, and the square piece was subjected to degreasing, acid washing, and Dy grain boundary diffusion treatment. The amount of Dy diffused was 0.8 wt%, the diffusion temperature was 900 °C, and the diffusion time was 15 h. The grain boundary diffusion in this example was conducted by a coating method to obtain a sintered neodymium-iron-boron magnet. The linear expansion coefficients of the product in different directions were tested using a thermomechanical analyzer, and the test results are shown in Table 4 below. The ramping rate was 5 °C/min, and the test temperature was 20-140 °C. In addition, the neodymium-iron-boron magnet obtained above was subjected to magnetic tests at 20 °C and 140 °C. The test results are shown in Table 5 below.

**Table 4. Linear expansion coefficients of neodymium-iron-boron products in Examples 1-2**

| | C1 (10⁻⁶/°C) | C2 (10⁻⁶/°C) | C3 (10⁻⁶/°C) | C4 (10⁻⁶/°C) | \|C1/C4\| |
|---|---|---|---|---|---|
| Example 1 | 5.56 | -2.69 | -2.93 | -2.71 | 2.05 |
| Example 2 | 5.31 | -2.88 | -3.04 | -2.96 | 1.79 |

**Table 5. Magnetic property results of neodymium-iron-boron products in Examples 1-2**

| | Br(T) 20°C | Hcj(kA/m) 20°C | Hej(kA/m) 140°C | Hcj temperature coefficient |
|---|---|---|---|---|
| Example 1 | 1.36 | 1569 | 559 | -0.536 |
| Example 2 | 1.343 | 2209 | 960 | -0.471 |

As can be seen from Example 2, after the blank prepared in Example 1 was subjected to heavy rare earth diffusion, C1, C2, C3, C4, and |C1/C4| were all within the patent ranges. Moreover, when the blank prepared in Example 1 was subjected to heavy rare earth diffusion, the product properties were greatly improved, showing better temperature resistance.

### Example 3

Other steps were the same as those in Example 1, except for the treatment process after completion of hydrogen absorption. The dehydrogenation temperature was 350 °C, the argon pressure introduced after completion of the dehydrogenation was 30 kPa, the heat preservation temperature was 800 °C, and the argon pressure introduced during the cooling at a temperature of not less than 350 °C was 30 kPa. The expansion coefficients of the tested product are shown in Table 6, and the corresponding product properties are shown in Table 7.

**Table 6. Linear expansion coefficients of neodymium-iron-boron product in Example 3**

| | C1 (10⁻⁶/°C) | C2 (10⁻⁶/°C) | C3 (10⁻⁶/°C) | C4 (10⁻⁶/°C) | \|C1/C4\| |
|---|---|---|---|---|---|
| Example 3 | 6.98 | -0.71 | -1.25 | -0.98 | 7.12 |

**Table 7. Magnetic property results of neodymium-iron-boron product in Example 3**

| | Br(T) 20°C | Hcj(kA/m) 20°C | Hej(kA/m) 140°C | Hcj temperature coefficient |
|---|---|---|---|---|
| Example 3 | 1.358 | 1544 | 547 | -0.538 |

### Example 4

Other steps were the same as those in Example 1, except for the treatment process after completion of hydrogen absorption. The dehydrogenation temperature was 250 °C, the argon pressure introduced after completion of the dehydrogenation was 35 kPa, the heat preservation temperature was 700 °C, and the argon pressure introduced during the cooling at a temperature of not less than 350 °C was 20 kPa. The expansion coefficients of the tested product are shown in Table 8, and the corresponding product properties are shown in Table 9.

**Table 8. Linear expansion coefficients of neodymium-iron-boron product in Example 4**

| | C1 (10⁻⁶/°C) | C2 (10⁻⁶/°C) | C3 (10⁻⁶/°C) | C4 (10⁻⁶/°C) | \|C1/C4\| |
|---|---|---|---|---|---|
| Example 4 | 6.73 | -0.77 | -1.22 | -1.0 | 6.73 |

**Table 7. Magnetic property results of neodymium-iron-boron product in Example 4**

| | Br(T) 20°C | Hcj(kA/m) 20°C | Hej(kA/m) 140°C | Hcj temperature coefficient |
|---|---|---|---|---|
| Example 4 | 1.361 | 1548 | 546 | -0.539 |

The above examples illustrate the embodiments of the present disclosure. However, the claimed scope of the present disclosure is not limited to the embodiments described above. Any modification, equivalent replacement, improvement, and the like made by those skilled in the art without departing from the spirit and principle of the present disclosure shall fall within the protection scope of the present disclosure.

## Claims

1. A high-temperature-resistant sintered neodymium-iron-boron magnet, wherein the magnet is represented by R-Fe-B-M and comprises, based on a mass ratio of 100%,
29 wt% to 35 wt% of R, wherein R is a rare earth element;
0.9 wt% to 1.3 wt% of B;
less than 5 wt% of M, wherein M is selected from one or more of Ti, V, Cr, Mn, Co, Ga, Cu, Si, Al, Zr, Nb, W, and Mo;
the balance is iron and inevitable impurities.

2. The magnet according to claim 1, wherein a linear expansion coefficient C1 parallel to a magnetizing direction of the magnet is (5 to 8) × 10⁻⁶/°C;
preferably, a linear expansion coefficient C2 perpendicular to the magnetizing direction and parallel to a pressing direction is (-3 to -0.6) × 10⁻⁶/°C;
preferably, a linear expansion coefficient C3 in the other direction perpendicular to the magnetizing direction is (-4 to -1) × 10⁻⁶/°C;
preferably, a mean value C4 of the linear expansion coefficients in two directions perpendicular to the magnetizing direction is (-3.5 to -0.8) × 10⁻⁶/°C, wherein C4 = (C2 + C3)/2;
preferably, 1.5 ≤ |C1/C4| ≤ 8.

3. A preparation method for the magnet according to claim 1 or 2, comprising:
(1) preparing an R-Fe-B-M alloy flake from respective starting materials by a rapid hardening and strip casting method;
(2) subjecting the alloy flake to hydrogenation treatment by introducing hydrogen; after completion of the hydrogenation treatment, performing heating to a temperature of 250 to 350 °C for dehydrogenation treatment; after completion of the dehydrogenation, introducing argon to not less than 30 kPa, and performing heating and heat preservation; after completion of the heat preservation, performing cooling to obtain an alloy powder;
(3) subjecting the alloy powder in step (2) to jet milling to obtain a magnetic powder, and performing pressing, sintering, and tempering treatments to obtain the magnet.

4. The method according to claim 3, wherein in step (2), a hydrogen absorption pressure for the hydrogenation treatment is 100 to 200 kPa, and a hydrogen absorption time is 30 to 180 min; preferably, in step (2), the dehydrogenation time is 180 to 360 min.

5. The method according to claim 3 or 4, wherein in step (2), argon is introduced to 30-60 kPa after completion of the dehydrogenation;
preferably, in step (2), a heat preservation temperature is 700-800 °C; a heat preservation time is 60 to 180 min;
preferably, in step (2), during the cooling, an argon pressure is ≥ 20 kPa at a temperature of not less than 350 °C.

6. The method according to any one of claims 3-5, wherein in step (3), the alloy powder in step (2) is mixed with a lubricant and subjected to jet milling to obtain a magnetic powder;
preferably, in step (3), a granularity D50 of the magnetic powder is 2 to 5 µm;
preferably, in step (3), a content of the lubricant is 0.03 to 0.5 wt% of the alloy powder in step (2).

7. The method according to any one of claims 3-6, wherein in step (3), the magnetic powder is press-molded under a magnetic field orientation; preferably, the orientation magnetic field is 1.5 to 2.5 T; preferably, in step (3), a sintering temperature is 800 to 1200 °C, and a heat preservation time is 3 to 20 h.

8. The method according to any one of claims 3-7, wherein in step (3), the tempering treatment is two-stage tempering, for example, two-stage tempering in a vacuum tempering furnace; a primary tempering temperature is 700 to 900 °C, and a heat preservation time is 3 to 7 h; a secondary tempering temperature is 450 to 600 °C, and a heat preservation time is 3 to 7 h.

9. The method according to any one of claims 3-8, further comprising step (4): performing grain boundary diffusion treatment on the magnet, wherein a diffusion source is at least one of heavy rare earth Dy, Tb, Ho, Nd, and Pr;
preferably, in step (4), a content of the diffused heavy rare earth is 0.1-1.5 wt%;
preferably, in step (4), a diffusion temperature is 800 to 950 °C, and a diffusion time is at least 3 h.

10. Use of the magnet according to claim 1 or 2 in the fields of new energy automobile industry and wind power generation.
